

Oct. 22, 1957

D. E. TILL ET AL

2,810,426

# RETICULATED WEBS AND METHOD AND APPARATUS FOR THEIR PRODUCTION

Filed Dec. 24, 1953



斐氏圖-2



一

1

2,810,426

**RETICULATED WEBS AND METHOD AND APPARATUS FOR THEIR PRODUCTION**

Derek E. Till, Concord, and Carl R. Smallman, Wollaston, Mass., assignors, by mesne assignments, to American Viscose Corporation, Philadelphia, Pa., a corporation of Delaware

Application December 24, 1953, Serial No. 400,252

20 Claims. (Cl. 154—27)

This invention relates to fibrous bodies and more particularly to reticulated webs or structures formed of fibrous materials and to methods and apparatus for preparing such bodies or structures.

Fibrous bodies or structures of fiber-forming organic substances are generally formed from filaments prepared by either extruding the fiber-forming organic substance through an orifice or by spraying the organic substance by the use of spray guns and the like. Methods which involve the extrusion of the fiber-forming substance through orifices are limited to the use of certain substances which may be filtered and which possess certain other characteristics, including wet and dry tensile strengths, necessary for the spinning operations. The filaments produced by conventional extrusion methods are continuous filaments and the size or denier is limited by the extrusion characteristics of the substance or of the spinning solutions of the particular substance. In many instances, it is desirable to incorporate various solid materials, such as fillers, into the fibers or filaments. However, it is not practical to do so when the material is to be extruded through fine orifices and the amount of foreign material which may be incorporated in the fiber or filament is strictly limited. In the production of sheet material or padding from such filamentary materials, it is necessary to collect the filaments and cut them to staple lengths. The staple is subsequently processed on conventional textile and felting equipment to form a woven sheet or felted layer or mat. Where the filament is formed of a potentially adhesive substance and it is desired to produce a product, with or without non-adhesive fibers, wherein the fibers are bonded together at their points of contact, it is necessary to subject the sheet or mat, as formed, to an activating treatment whereby the potentially adhesive fibers become tacky or adhesive and are capable of bonding to other fibers at their points of contact and then deactivate the fibers.

As an alternative, fibers or filaments may be formed from a wide range of substances by the use of various types of spray guns. Because of the relatively large size of the spray gun orifices as compared to extrusion orifices such as those of a rayon type spinneret, for example, the limitations with respect to the characteristics of the spinning liquid are far less exacting than for the extrusion methods. Various materials such as fillers, hardening agents, plasticizing agents and the like may be incorporated in the spinning liquids. If it is desired to form a product of potentially adhesive fibers and non-adhesive fibers, the potentially adhesive fibers may be produced by spraying into an air stream containing air-borne non-adhesive fibers and collecting the mixed fibers, for example as shown in the patent to Carleton S. Francis, Jr., No. 2,357,392.

In the copending application of Howard O. McMahon and Paul C. Watson, Serial No. 400,240, filed December 24, 1953, there is disclosed a method for the production of reticulated fibrous webs of elastomeric material. In

2

the copending application of Paul C. Watson, Serial No. 400,239, filed December 24, 1953, there is disclosed a method for the production of reticulated fibrous webs of non-elastomeric thermoplasts. In the methods disclosed in these copending applications, a fiber-forming spraying liquid such as a solution or dispersion of the elastomer or thermoplastic in a suitable solvent, or the molten fiber-forming material is extruded into a high velocity stream of gas as a relatively large-diameter stream of plastic. The high velocity stream of gas attenuates the plastic stream and breaks the attenuated stream transversely to form the fibers. When certain thermoplastic-containing solutions are employed as the spraying liquid, it is possible that the extruded stream of plastic is also fibrillated by the high velocity stream of gas, that is, the stream of plastic is split lengthwise. The gas stream at least partially removes the solvent or partially cools the molten plastic and thereby partially sets the fiber-forming material. Fibers of the partially set fiber-forming material are in an adhesive condition, that is, they are in a sticky cementitious, agglutinous, or tacky condition and readily adhere to each other upon contact.

The newly formed fibers are carried by the gas stream to a suitable collecting surface or a secondary stream of gas may be employed to float or carry the fibers to the collecting surface. While the fibers are thus carried, they come into contact with each other particularly in the case of the fibers formed of elastomeric materials and the fibers may become intertwined to form rope-like or string-like fibers of appreciable size without actually coalescing. The reticulated mat or sheet formed by collecting the fibers consist of fibers or fiber-like bodies whose transverse or cross-sectional dimensions vary over a considerable range.

One of the purposes of the present invention is to provide an improved method for the production of fibers and reticulated fibrous products.

Another purpose of this invention is to provide a method for the production of fibers of relatively uniform cross-sectional dimensions and to produce reticulated fibrous products wherein the fiber size lies within a relatively narrow range.

A further purpose of the invention is to provide apparatus for the production of reticulated fibrous products.

A specific purpose of the present invention is to provide a method and apparatus for the production of fibers by a spraying technique wherein the intertwine or roping of the fibers is substantially eliminated.

Other objects and advantages of this invention will become apparent from the disclosure and claims which follow.

In the drawings,

55 Figure 1 is a diagrammatical elevational view partially in section of one form of apparatus for the preparation of reticulated fibrous products.

Figure 2 is a diagrammatical elevational view partly in section of a further form of apparatus for the products 60 of this invention.

The present invention contemplates inducing an electrical charge on fibers immediately upon their being formed by the spraying techniques disclosed in the aforementioned applications. The fibers are formed by extruding a fiber-forming spraying liquid as a relatively large diameter stream of plastic into a high velocity stream of gas and under the influence of a high potential electrostatic field. The stream of plastic is charged electrically, attenuated and broken transversely and may be fibrillated into a plurality of fibers within or under the influence of the electrostatic field. The fibers are then collected upon a collecting surface which carries an elec-

trical charge opposite that of the charge carried by the fibers, or a porous collecting surface may be interposed between the area of fiber formation and an electrode having a charge opposite that of the fibers.

Unlike dry spinning, as performed in the rayon and synthetic fiber industries, in which a spinneret with multiple minute holes is used to produce a predetermined number of filaments each substantially of the same size as the holes and in which the continuous filaments are pulled continuously from the face of the spinneret to a moving collector, the spraying process of the invention utilizes a single relatively large extrusion orifice producing a single large-diameter plastic stream which is attenuated and possibly fibrillated into a multiplicity of fibers and fibrils, the diameters of which fibers and fibrils are small fractions of the orifice diameter, there being no continuous filament running between the orifice and the collector.

The velocity of the gas into which the spraying liquid is extruded is appreciably higher than the velocity of extrusion of the spraying liquid and the direction of extrusion is coincident with the direction of the gas flow. The high velocity stream of gas thereby attenuates and possibly fibrillates the spraying liquid, that is, the stream of liquid is highly attenuated and may be split lengthwise into two or more thinner fibers or fibrils and is broken up into discontinuous fibers or fibrils of varying length by the high velocity gas.

Immediately upon extrusion of the spraying liquid and the on-set of fiber formation an electrostatic charge is induced on the stream of plastic and on the fibers. This charge aids in fibrillation of the stream of plastic. Each of the fibers thus formed carries a like charge and the individual fibers thereby repel each other.

The stream of gas partially or substantially completely sets the fiber-forming material due to a partial or substantially complete vaporization of the solvent or to a cooling of the spraying liquid to form the electrically charged, discontinuous, attenuated fibers or fibrils. The gas also carries, supports or floats the fibers or fibrils and finally deposits them or allows them to deposit upon a suitable collecting surface. Alternatively, a low velocity or secondary stream of gas may be provided having a velocity lower than that of the high velocity or primary stream of gas but having a sufficiently high velocity so as to carry, support or float the fibers and fibrils and finally deposit them or allow them to deposit upon a suitable collecting surface. The collecting surface may carry a charge opposite that of the charge induced upon the fibers to thereby attract the fibers. Alternatively, a charged electrode may be positioned behind a collecting surface so that the fibers are arrested in their travel toward the attracting electrode and will be collected in a charged form. The fibers may be collected in either a substantially set or dry non-adhesive condition whereby the product is a loose fluffy mat or web or the fibers may be collected in an adhesive or tacky condition whereby they become bonded together at their points of contact to provide a coherent reticulated web or sheet.

Our invention is applicable to the production of fibers and fibrous mats or webs from rubber, both natural rubbers and synthetic rubbers or rubber substitutes. Such elastomeric materials or rubbers, both natural and synthetic, which are soluble in inexpensive, volatile organic solvents are well suited for the production of the reticulated mats or webs of this invention. Elastomeric materials satisfactory for use in the herein described method include natural rubbers such as crepe rubber and synthetic rubbers or rubber substitutes such as chloroprene polymers, for example, neoprenes; butadiene-acrylonitrile copolymers known as Buna-N, for example, Butaprene, Paracril, Ameripol-D, Perbunan, Chemigum, and Hycar-OR; butadiene-styrene copolymers, for example, Ameripol-F, Hycar-OS and GR-S; isoprene-isobutylene

copolymers, for example, GR-I and butyl; and organic polysulfides, for example, Thiokol. Mixtures of specific elastomeric materials may be utilized to provide desired characteristics. The specific elastomers are enumerated merely as illustrative and are not intended as limitations of the invention.

10 The spraying or fiber-forming liquid may be formed by dissolving the fiber-forming elastomeric material in a satisfactory organic solvent such as aliphatic and aromatic hydrocarbons, chlorinated hydrocarbons, aralkyl hydrocarbons and the like, those being preferred which will volatilize readily at moderately elevated temperatures. The solvent utilized in forming the spraying liquid will be dependent upon the specific elastomer and upon characteristics desired in the spraying liquid such as volatility of the solvent. For example, solvents which are satisfactory include benzene, naphtha, toluene, xylene, cyclohexanone, ethylene chloride, methylene chloride, carbon tetrachloride, nitroparaffins, ketones and the like. Such inexpensive volatile organic solvents as benzene and naphtha are entirely satisfactory for use in fiber-forming liquids containing natural rubber. The spraying liquids may contain from about 5% to about 50% of the fiber-forming elastomeric material and preferably contain between about 10% and about 35% rubber or rubber substitute.

20 Gas-forming or blowing agents such, for example, as ammonium carbonate, sodium acid carbonate, diazo-aminobenzene and the like, may be added to the elastomeric materials or spraying liquids, if desired. These agents include solids and gases and are commonly employed in the production of sponge rubber and porous rubber sheet and products. They are adapted to release or form a gas such as ammonia, carbon dioxide or other inert gas at a temperature at which the elastomeric material is cured or vulcanized.

30 The properties and characteristics of the fibers formed from the elastomeric materials may be varied as desired by incorporating additives in the spraying liquid. Substances such as normally employed in preparing finished rubber articles from crude natural rubbers or synthetic rubbers may be added, for example, carbon black, curing or vulcanizing agents such as sulfur, accelerator, antioxidants, plasticizers and the like. Detackifying agents, such as paraffin wax, stearic acid and the like may be incorporated in the spraying liquid so as to decrease the natural adhesive or tacky nature of the unvulcanized fibers. Coloring agents, such as dyes and pigments may be utilized to produce fibers having desired colors or tints. Abrasive particles such as emery dust, Carborundum, silica, etc., may be incorporated in the spraying liquid to provide products having abrasive properties. Fillers such as clay, whiting, kaolin, French chalk and the like may be added to impart desired characteristics and to reduce the cost of the fibers. The amount of the additive may be varied over a wide range as desired. In the case of solid fillers, from about 50% to about 150% filler, such as clay, finely divided pigments and the like, based upon the weight of the elastomer, may be incorporated in the spraying liquid. Lesser or greater amounts, however, may be employed depending upon the type of product desired.

40 The additive substances may be mixed with the elastomer as by milling the elastomer and the additive, or the additive substance may be mixed with or dispersed in the solution of the elastomer. By varying the amount of solvent and the amount of additive substances and the degree of milling, the viscosity of the spraying liquid may be varied over an extremely wide range. It is possible to utilize spraying liquids in forming the products of this invention which are totally unsuited for use in the usual or conventional spinning methods.

50 The primary gas stream may be at normal atmospheric temperatures or any other desired temperatures. For

example, the temperature may be elevated so as to increase the rate of volatilization of the solvent. The gas may consist of a chemically reactive gas, steam, air or other inert gas such as nitrogen, carbon dioxide and the like. Since the fibers as they are formed by the attenuating effect of the gas stream and the volatilization of the solvent are tacky or cementitious, solid particles or short preformed fibers may be introduced into the primary gas stream so as to provide a coating on the fibers. For example, a detackifying agent such as talc, wood flour, starch, etc., may be introduced to provide a coating which decreases or destroys the natural tackiness of the fibers and allows the collection of the fibers in a body wherein there is little or no adhesion between the crossing filaments. Short, preformed fibers either synthetic or artificial such as viscose rayon staple, cotton, wool, asbestos, etc., or finely divided particles such as leather, rayon flock, cork dust and the like may be introduced if desired.

The invention is also applicable to the production of fibers and reticulated fibrous webs or mats from fiber-forming, non-elastomeric thermoplast which are primarily synthetic, non-elastomeric polymers capable of forming fibers from volatile organic solvent solutions or from hot melts or both, and are thermoplastic or may exist in a thermoplastic state. The spraying liquids comprised of the solvent solutions of the synthetic polymers or the hot melts of the polymers or both are capable of being attenuated and fibrillated to form the fibers. The fibers of the polymer are capable of being rendered adhesive, sticky, cementitious, agglutinous or tacky by heating to temperatures elevated with respect to normal or room temperatures or by treatment with a solvent or both, and the polymers and fibers formed therefrom may therefore be termed "potentially adhesive materials."

The non-elastomeric thermoplasts satisfactory for the purposes of this invention consist of a wide variety of substances selected generally from the classes or groups consisting of organic cellulose derivatives, thermoplastic resins and thermosetting resins in their thermoplastic state. These thermoplasts include organic solvent soluble cellulose esters such as cellulose acetate, cellulose acetate-butylate and the like; organic solvent soluble cellulose ethers such as ethyl cellulose, and the like; vinyl resins, which may be defined as solid, thermoplastic, saturated synthetic resins resulting from the polymerization of compounds containing the vinyl group such as polyvinylchloride, copolymers of vinyl chloride and vinyl acetate (Vynon), copolymers of vinyl chloride and acrylonitrile (Dyne), polyacrylonitrile including copolymers of polyacrylonitrile (Acilan, Orlon), polystyrene, polyacrylates such as ethyl acrylate polymers, methyl acrylate polymers and the like; polyesters (Dacron); polyamides (nylon), including alcohol soluble nylon; organic solvent soluble thermosetting resins of the types which are capable of existing in a thermoplastic state such, for example, as urea-formaldehyde, melamine-formaldehyde, thiourea-formaldehyde, glyptals, silicones and the like, which resins are attenuated and fibrillated while they are in their thermoplastic state and which, if desired, may be converted subsequently to the thermoset state while in fiber form; and the like. Mixtures of specific thermoplasts may be utilized to provide fibers and structures of desired characteristics. The specific thermoplasts are enumerated merely as illustrative and are not intended as limitations of the invention.

The spraying liquid may be formed by dissolving the fiber-forming thermoplast in a suitable organic solvent which may be volatilized at moderately elevated temperatures, or the spraying liquid may comprise a hot melt or molten mass of the thermoplast. For example, a spraying liquid may comprise a solution of Vynon in tetrahydrofuran and methyl isobutyl ketone, or an alcohol solution of alcohol soluble nylon, or a hot melt of nylon. Where the spraying liquid comprises a solution

of a thermoplast, the solution may contain from about 10% to about 55% of the fiber-forming thermoplast, the specific solids content varying with the different types of fiber-forming materials.

5 The properties and characteristics of the fibers formed from the thermoplasts may be varied as desired by incorporating additives in the spraying liquid. For example, fillers, coloring agents such as dyes and pigments, plasticizers and the like may be incorporated in the solution of the thermoplast or in the hot melt. By varying the relative proportions of solvent, thermoplast and additive substance, the viscosity of the spraying liquid may be varied over a wide range. It is possible to utilize spraying liquids in forming the products of this invention which are totally unsuited for use in the usual or conventional spinning methods.

The gas streams for attenuating the plastic stream and carrying the fibers, may be at normal atmospheric temperature or at any other desired temperature. For 10 example, the temperature may be elevated so as to increase the rate of volatilization of the solvent. Any desired gas may be employed such as air, nitrogen, carbon dioxide, steam and the like.

The elastomers and thermoplasts are potentially adhesive materials, as described hereinbefore. Since the fibers as they are formed are adhesive or tacky, a reticulated web or structure can be produced by collecting them on a surface, or a composite reticulated web or structure can be produced by collecting them in combination with other particulate material such as preformed fibers and/or discrete particles, preferably of a non-adhesive, non-elastomeric material, which may be introduced into the streams of gas. The preformed fibers or discrete particles are thereby brought into contact with the potentially adhesive fibers while the latter are in a tacky or cementitious condition and the preformed particulate material adheres to the newly formed fibers. The fibers may be collected while they are in an adhesive condition or afterwards. The fibers as 20 collected are deposited in a completely random distribution or haphazard manner to produce a reticulated, web or structure. Where the fibers are collected while they are in a tacky condition, the fibers will stick together where they contact each other and where they contact 25 preformed particulate material, if such material is present. The fibers may be collected after complete removal of the solvent or a cooling of the fibers to a temperature at which they are not tacky in which case they will not stick together. The degree of bonding of the fibers in 30 the reticulated web may be thus controlled as desired. Conventional methods of handling staple fibers, even though elaborate carding equipment is employed, do not produce webs having the totally random distribution of fibers as formed by this method. This method also 35 eliminates the activating procedure required where conventional methods are utilized in forming the mixed fiber or composite bodies.

The term "particulate non-adhesive material" is used to designate preformed fibers and/or discrete particles 40 of a material which is not rendered adhesive or tacky under the conditions at which the elastomers and thermoplasts are adhesive.

Among the non-adhesive substances or materials which may be employed in forming the composite bodies 45 are natural fibers, such for example as wood fibers, cotton, flax, jute, sisal, kapok, wool, hair, and silk, other natural substances such as leather and cork; synthetic fibers, for example, cellulosic fibers such as cellulose hydrate, cellulose derivatives such as cellulose esters, mixed cellulose esters, cellulose ethers, mixed cellulose ester-ethers, mixed cellulose ethers, cellulose hydroxy-alkyl ethers, cellulose carboxyalkyl ethers, cellulose ether-xanthates, cellulose xantho-fatty acids, cellulose thiourethanes, fibers made of alginic acid, gelatine, casein; 50 mineral fibers such as spun glass, asbestos, mineral wool

and the like; and fibers made of natural and synthetic resins which are not rendered tacky when the potentially adhesive thermoplastic fibers or fibrils are rendered tacky; also fibers and filaments made by slitting, cutting or shredding non-fibrous films, such as waste cellophane. In addition to or in lieu of the preformed fibers, preformed discrete particles of natural and synthetic materials may be introduced into one or both of the streams of gas; for example, cork dust, leather dust, wood flour, flake particles, fibers of floc length and the like. Two or more different non-adhesive materials may be introduced into the gas streams and the different materials may be of different physical form; for example, one may be in fiber form and another in powdered form, depending upon the nature and characteristics desired in the final product. In producing composite webs or structures including preformed non-adhesive fibers, it is preferable to employ both the primary and secondary streams of gas and introduce the preformed fibers into the secondary air stream. Preformed discrete particles may be introduced into either gas stream. Where the composite body is to include both preformed fibers and discrete particles, the discrete particles, for example, cork dust or wood flour, may be introduced into the primary stream of gas and the preformed fibers, for example, wood fibers, rayon staple or mineral wool fibers, may be introduced into the secondary stream of gas. Both types of preformed non-adhesive material, however, may be introduced into the primary or high velocity stream of gas or into the secondary stream of gas.

The method of the present invention may be practiced by the use of apparatus as illustrated more or less diagrammatically in Figure 1. A tower or chamber 1 open at its upper end is provided with means such as a blower 2 for passing a gas at a relatively low velocity through the tower. At or adjacent the base of the tower, there is mounted a spraying unit 3 which comprises a spraying liquid or spray tube 4 having an extrusion orifice at its upper end, the other end communicating with a liquid conduit 5 through which the spraying liquid is passed under pressure. Surrounding the spraying liquid tube 4 there is positioned a gas nozzle 6, the spray tube 4 extending beyond the end of the gas nozzle so as to position the extrusion orifice in the path of the gas issuing from the nozzle. The gas nozzle is connected with suitable means such as a blower 7 for passing a gas through the nozzle at a relatively high velocity. The spraying unit is preferably mounted concentrically with respect to the walls of the tower or chamber. A collecting surface such as a conveyor screen 8 is positioned across the open end of the tower. An open ended cylinder 9 is mounted in spaced relationship with respect to the spraying unit 3 as by means of insulation 10. Sources of high potential 11 and 11a such as generators having a capacity of from about 5,000 volts to about 50,000 volts are connected electrically at one side to ground. The spraying unit 3 and tower 1 are also grounded. The cylinder 9 and the conveyor screen 8 are independently connected to the other side of the high potential sources.

The spraying liquid is extruded into the high velocity stream of gas in the form of a single relatively large diameter stream of plastic. The high velocity stream of gas draws or attenuates the spraying liquid and breaks the stream transversely into discontinuous lengths to form a plurality of fibers of varying length. In some instances, the high velocity stream of gas may possibly fibrillate the stream of plastic, that is, split the stream lengthwise into two or more thinner streams. The velocity of extrusion and the velocity of the stream of gas may be varied so as to regulate the amount of attenuation and to regulate the length of the fibers and for those spraying liquids which may be fibrillated, the relative velocity of the stream of gas with respect to the velocity of extrusion may be increased to cause fibrilla-

tion. Solvent is evaporated simultaneously with the attenuation action so as to partially set or harden the fiber-forming material or if the spraying liquid comprises a hot melt, the partial setting or hardening is accomplished by a partial cooling of the attenuated stream.

Simultaneously, with the extrusion and with the filament formation under the influence of the electrostatic field, an electrical charge is induced upon the filaments, the charge being opposite that applied to the charging cylinder 9. Since all of the fibers thereby carry the same induced charge, they will repel each other and prevent or eliminate intertwining or roping of the fibers during their travel in the air stream.

The charged fibers or fibrils are carried or floated in the gas stream and are also carried towards the target by the attractive forces produced by the difference in potential between the fibers and the collecting surface, which may be grounded or preferably carries a charge opposite to that of the fibers. Solvent continues to volatilize from the fibers or the cooling of the molten fibers continues during the passage of the fibers to the collecting surface where the fibers are finally deposited or collected. As the fibers collect on the screen or other porous or foraminous surface, the resistance of the reticulated web or mat 12 to the passage of gas increases and for the production of thicker webs or mats, a suction chest 13 may be positioned on the opposite side of the porous collecting surface or screen. The suction chest may also serve as an aid to the recovery of vaporized solvent, if desired. In some instances, particularly in the production of reticulated webs and mats of the elastomeric materials, it is desirable to utilize a secondary stream of gas which may be supplied by the blower 2 and which surrounds or envelops the primary stream of gas. The secondary stream of gas is passed through the chamber or tower at a lower velocity than the primary or high velocity stream of gas and serves to carry or float the fibers to the collecting surface and also complete the removal of solvent and the setting of the fibers. The gas streams may be at any desired temperature so as to regulate the condition of the fibers at the time of collection on the collecting surface. By increasing the gas temperatures, the fibers may be deposited in a substantially non-adhesive condition.

The characteristics of the reticulated mat or web may be varied by altering the positioning of the collecting surface with respect to the spraying unit. By decreasing the distance between the collecting surface and the spraying unit, the distance through which the fibers travel before being collected is also decreased. The fibers have had a shorter period to become set and are accordingly deposited in a more tacky condition to form a more thoroughly bonded mass. The velocity of the fibers at the instant of deposition is higher the shorter the distance of travel and, hence, the mat or web will be of higher density. By increasing the distance between the collecting surface and the spraying unit, the fibers will be in a less tacky condition and will be deposited at a lower velocity and the web or mat is lower in density and the fibers are less firmly bonded together.

In production of fibrous webs or mats utilizing the present method, the collecting surface or screen may be spaced from about 3 feet to 10 or 12 feet from the spraying unit depending upon the film-forming material, the specific spraying liquid, the spraying conditions, and the type of product desired.

The reticulated web or mat may be passed through a heating chamber 14 before being removed from the collector screen by a doctor blade or doffer 15. The heating chamber 14 may be employed to activate the fibers to provide a greater bond between them or in the case of elastomeric fibers the heating chamber may be employed to effect a curing or vulcanization of the elastomer. For the production of thin sheet-like products, the reticulated web upon activation of the fibers may be passed between pressure rolls 16 or the pressure rolls may be provided with

desired protuberances to provide additional bonding at predetermined localized areas. The heater may be replaced by heated pressure rolls. The reticulated web is finally accumulated on the take-up roll or drum 17.

In the production of fibrous bodies comprising preformed non-adhesive fibers and/or discrete particles and the potentially adhesive fibers formed as described, the preformed non-adhesive fibers and/or discrete particles are preferably carried in a secondary stream of gas and may be introduced through the blower 2. The non-adhesive fibers or particles are thereby carried or blown into contact with the fibers while these latter fibers are in a partially set and tacky or cementitious condition and thereby become firmly attached to the sprayed fibers. The spraying conditions are maintained so that the sprayed fibers are still in a somewhat tacky condition when they are collected on the conveyor screen 8.

Although the chamber or tower 1 is shown as being provided with a spraying unit consisting of a single spray tip and nozzle, it is to be understood that such illustration is merely for purposes of simplifying the drawing and the foregoing discussion. A plurality of spaced spraying units may be mounted within a large tower.

As illustrated in Figure 2, the tower 1, the spraying unit 3 and one side of the high potential source 11 are connected electrically to ground. The charging electrode or cylinder 9 and a second electrode 18 are connected electrically to the other sides of independent high potential sources. The fibers may be collected upon a porous or foraminous collecting surface 19 such as a porous flexible conveyor belt formed of an electrical insulating material which is interposed in the path of the fibers between the spraying unit 3 and charging electrode 9 and the second electrode 18 which may comprise a metallic plate. The collection of the fibers on the porous collector surface occurs as the fibers are arrested in their flow toward the electrode 18.

Although the apparatus as illustrated shows the spraying operation as being performed by establishing an upwardly directed high velocity stream of gas and extruding the fiber-forming liquid upwardly into the stream of gas. Equally satisfactory results and products may be produced by spraying downwardly or horizontally or in any other desired direction.

The spraying and fiber-forming method has been found to be particularly satisfactory and inexpensive for the production of reticulate webs and mats consisting of very fine fibers. Spraying liquids having a viscosity or apparent viscosity within a range of from about 150 C. P. S. to about 30,000 C. P. S. have been satisfactorily utilized in preparing reticulate webs and mats. The viscosity and the apparent stringiness of the spraying liquids do not appear to be a measure of the fiber-forming characteristics when utilized in the method of this invention. The size of the fibers may be controlled by varying the concentration of the fiber-forming material in the spraying liquid, by varying the side of the extrusion orifice, by varying the relative velocity of the high velocity stream of gas with respect to the velocity of extrusion of the spraying liquid and to some degree by varying the potentially applied charging electrode 9. As pointed out hereinbefore, the application of the charge to the fibers as they are formed substantially eliminates the intertwining and roping of the fibers during their travel to the collecting surface. We have also discovered that the fiber size is, in general, smaller than that of fibers produced without spraying under the influence of an electrostatic field and that the range of size is substantially reduced by the present method. Reticulate webs or mats prepared as described are more uniform and smooth in appearance than similar products prepared without inducing the electrical charge on the fibers.

It is well known that for certain types of gas filters it is essential to employ fine fibers, that is, fibers having a diameter of the order of 2 to 3 microns and lower.

Considerable difficulty is encountered in preparing filter media from such fine fibers because they cannot be handled by conventional commercial fiber and textile equipment thus rendering such media quite costly. The only known materials commercially available are certain grades of glass fibers and imported asbestos. No comparable organic fibers, either natural or synthetic, are available.

The present method provides an inexpensive reticulated filter medium of very fine fibers which is admirably suited for both gas and liquid filters, gas masks, and the like. The reticulated, fibrous bodies are also very highly effective as thermal and sound insulating materials. Because of the relatively light weight of the webs or mats, the bodies or structures are especially well suited for such uses as thermal and sound insulation for aircraft, thermal insulation for arctic clothing and the like. For example, reticulated webs, highly satisfactory for filter purposes have been prepared for spraying liquids containing Vinyon, polyacrylonitrile and Dynel. The fibers have had a diameter of less than 1 micron to about 3 microns with the large majority of the fibers having a diameter within the range of 1 to 3 microns.

In a small scale production of fibrous, reticulated mats or webs of this invention, a tower may be employed having a diameter of four feet and a height of about twenty-five feet. The spraying unit 3 consisting of a spinning tip 4 and a nozzle 6 is mounted concentrically within the tower at a point from about 3 feet to about 15 feet from the collecting screen. If the filament-forming material is to be extruded downwardly, the spraying unit may be mounted adjacent or at the top of the tower. A plurality of spaced spraying units may be employed if desired.

A blower may be provided to introduce an inert gas such as air at the bottom of the tower and suitable heating means may be provided to permit regulation of the temperature of the air stream if a secondary stream of gas is employed. The collecting conveyor may consist of a suitable screen such as a screen formed of Saran. The spray or extrusion orifice for the thermoplasts may be varied. Orifices between about 0.01 inch and about 0.05 inch in diameter have been satisfactory. The primary gas stream or high velocity gas stream may be provided through a nozzle having an internal diameter of from about 0.25 inch to about 0.75 inch. The extrusion orifice is positioned from about 0.25 inch to 1 inch beyond the terminus of the nozzle. The thickness of the reticulated web or mat is controlled by regulating the speed of the collecting conveyor.

For example, reticulated fibrous webs have been produced in a tower as described above in which the collecting screen was spaced about 4 feet from the spraying unit. The orifices through which the fiber-forming liquid was extruded, had a diameter of about 0.010 inch and the internal diameter of the gas nozzles was about 0.25 inch. Four spraying units were employed with a spacing of about 1.5 inches between adjacent extrusion orifices. The charging cylinder and collecting screen were maintained at a positive potential with respect to the spraying unit of about 20,000 volts. For example, a spraying liquid containing about 25% Vinyon in tetrahydrofuran was extruded at a velocity of about 100 feet per minute and air supplied to the gas nozzle at from 24,000 to 27,000 feet per minute. The reticulated web was formed by collecting the fibers without the use of a secondary stream of gas. The large proportion of the fibers had a diameter in the vicinity of 1 micron and microscopic examination showed that the fibers were relatively straight and within the range of a fraction of a micron to about 3 microns in diameter. The collected web was light in weight and fluffy with the fibers loosely bonded together and had a very smooth and warm feel.

In a similar manner, webs were produced by using a 21% solution of Dynel in dimethylformamide. The

fiber size was within the same range and like the Vinyon fibers, the fibers were relatively straight and uniform. Fibrous webs have also been prepared from spraying liquids containing from 10% to about 15% polyacrylonitrile dissolved in dimethylformamide. The individual fibers are very regular and smooth and appear to be of about the same diameter, namely about 1 micron.

In the production of similar products from elastomeric materials, the collecting surface is preferably spaced at least about 5 or 6 feet from the spraying unit. Extrusion orifices may vary in diameter depending upon the fiber size desired and the gas nozzle diameters may also be varied. We have employed satisfactorily spraying tubes having orifices up to about 0.06 inch in diameter and gas nozzles having diameters of up to about 0.75 inch. The extrusion orifice may extend from about 0.25 inch to about 1 inch beyond the terminus of the nozzle. It is also preferable to employ a secondary air stream because of the greater density of the individual fibers. The elastomeric materials may be combined with anti-oxidants, fillers, accelerators and coloring agents before dissolving or suspending in benzene or naphtha base solvents. Satisfactory products have been prepared from natural rubber, for example, pale crepe, and synthetic rubbers or rubber substitutes, for example, neoprene, by extruding the spraying liquids at a velocity from about 50 feet per minute to about 100 feet per minute. The primary or high velocity stream of air had a velocity of from about 20,000 to about 40,000 feet per minute. Secondary air velocities have been varied from about 500 to about 700 feet per minute.

The webs and mats formed by inducting an electrical charge on the plastic stream and the fibers have been more uniform in appearance and there is substantially no intertwining or roping of fibers apparent in the products. The fiber size is much more uniform as compared to similar products prepared without inducing a charge on the fibers as they are formed. In general, the fibers are of smaller diameters for the same spraying conditions as well as being more uniform when compared with fibers prepared without the influence of the electrostatic field.

Filters formed of the reticulated webs or mats of thermoplasts have exhibited filtration properties which are as satisfactory and in some cases of higher efficiency than the highest grade, commercially available filter materials formed of glass and mineral fibers. In general, these filter bodies have also exhibited an appreciably lower density than glass and mineral fiber filters. For example, a web of Vinyon fibers prepared as described herein having a density of 6 grams per square feet has substantially the same filtration efficiency as a web or mat of glass fibers having a density of 10 grams per square feet.

The following table is a representative comparison of filter sheets prepared in accordance with this invention and of two commercially available filter mediums when used to filter a 0.3 micron smoke:

Table I

|                         | Density<br>(gm./sq.<br>ft.) | Velocity<br>of gas<br>flow<br>(ft./min.) | Pressure<br>drop<br>(mm.<br>H <sub>2</sub> O) | Percent<br>Efficiency |
|-------------------------|-----------------------------|------------------------------------------|-----------------------------------------------|-----------------------|
| Vinyon.....             | 6                           | 20                                       | 1.8                                           | 18                    |
| Vinyon.....             | 12                          | 28                                       | 3.0                                           | 38                    |
| Dynel.....              | 6.5                         | 20                                       | 5.0                                           | 25                    |
| Glass Fibers.....       | 10                          | 20                                       | 2.5                                           | 20                    |
| Felt Filter (wool)..... | 46                          | 28                                       | 4.0                                           | 12                    |

Filter bodies of various thicknesses and density have been prepared and their efficiencies compared with the AEC absolute filter when using a 0.3 micron smoke (di-octyl phthalate vapor). The results of these tests are set forth in the following table:

Table II

|                             | Thickness<br>(inches) | Density<br>(gm./sq.<br>ft.) | Velocity<br>of gas<br>flow<br>(ft./min.) | Pressure<br>drop<br>(mm.<br>H <sub>2</sub> O) | Percent<br>efficiency |
|-----------------------------|-----------------------|-----------------------------|------------------------------------------|-----------------------------------------------|-----------------------|
| AEC Absolute<br>Filter..... |                       | 20                          | 20                                       | 100                                           | 99.9                  |
| Dynel.....                  | 0.024                 | 8.9                         | 28                                       | 59                                            | 97.5                  |
| Dynel.....                  | 0.041                 | 15.0                        | 28                                       | 103                                           | 99.6                  |
| Polyacrylonitrile.....      | 0.020                 | 7.5                         | 28                                       | 40                                            | 92.0                  |
| Do.....                     | 0.043                 | 17.0                        | 28                                       | 110                                           | 99.8                  |

The products of this invention are not limited to the use as gas filters but may be employed satisfactorily for any applications requiring low density, fibrous structures such as for the acoustical treatment of aircraft or similar applications where the weight of the sound attenuating or absorbing material must be kept to a minimum.

Obviously, the fibrous products are also highly satisfactory for applications where the weight need not be held at a minimum. The fibrous products are also highly efficient when utilized as thermal insulation as in aircraft, arctic clothing, and the like. The fibers may be employed for other purposes by collecting the fibers in a non-adhesive state so that the individual fibers may be readily separated from the collected mat or web. Such fibers may be employed in the preparation of the textile yarns and the like.

The products prepared from the elastomeric materials may be employed for a wide variety of uses such as the preparation of elastic fabrics for the manufacture of wearing apparel such as foundation garments, bathing suits and the like. For these purposes the products may be employed either in the form of a reticulated, fibrous rubber web or sheet or in the form of composite structures wherein the fibrous web is combined with a textile material. The fibrous web of the elastomeric material may also be utilized as a fibrous web or in the form of a composite structure for use as belting, girdles, garters and the like. The fibrous webs of elastomeric materials may be secured to or combined with sponge or foam rubber sheets to reinforce the foam or sponge rubber. Other uses will occur to those skilled in the art.

It is to be understood that changes and variations may be made without departing from the spirit and scope of the invention as defined in the appended claims.

It is to be further understood that the specific examples have not been set forth as limitations but merely to illustrate the invention.

We claim:

1. The method of producing a reticulated, fibrous body which comprises providing a fiber-forming liquid containing a potentially adhesive, fiber-forming organic material selected from the group consisting of thermoplasts and elastomeric materials; establishing an electrostatic field of high potential; establishing a high velocity stream of gas; discharging the stream of gas into the ambient atmosphere within the electrostatic field; extruding the fiber-forming liquid into and within the stream of gas at a point beyond the point of discharge of the stream of gas and under the influence of the electrostatic field to induce an electrical charge on the extruded liquid, the direction of extrusion being coincident with the direction of the gas flow; attenuating the extruded fiber-forming liquid, breaking the attenuated fiber-forming liquid into discontinuous lengths and at least partially setting the fiber-forming liquid to form discontinuous, electrically charged fibers by maintaining the velocity of the stream of gas at the point of discharge at a value greater than the velocity of extrusion of the fiber-forming liquid; and collecting the discontinuous fibers in random distribution to form a reticulated, sheet-like fibrous body.

2. The method as defined in claim 1, wherein the fiber-forming liquid comprises a solution of a thermoplast.

3. The method as defined in claim 1 wherein the fiber-forming liquid comprises a molten thermoplastic.

4. The method as defined in claim 1 wherein the fiber-forming liquid comprises a solution of a vinyl resin.

5. The method as defined in claim 1 wherein the fiber-forming liquid comprises a solution of a copolymer of vinyl chloride and vinyl acetate.

6. The method as defined in claim 1 wherein the fiber-forming liquid comprises a solution of a copolymer of vinyl chloride and acrylonitrile.

7. The method as defined in claim 1 wherein the fiber-forming liquid comprises a solution of a polyacrylonitrile.

8. The method as defined in claim 1 wherein the fiber-forming liquid comprises a solution of an elastomeric material.

9. The method as defined in claim 1 wherein the fiber-forming liquid comprises a solution of a natural rubber.

10. The method as defined in claim 1 wherein the fiber-forming liquid comprises a solution of a synthetic rubber.

11. The method as defined in claim 1 wherein the fibers are collected on a surface having an electrical charge opposite the electrical charge carried by the fibers.

12. The method of producing a reticulated, fibrous body which comprises providing a fiber-forming liquid containing a potentially adhesive, fiber-forming organic material selected from the group consisting of thermoplasts and elastomeric materials; establishing an electrostatic field of high potential; establishing a primary high velocity stream of gas; discharging the stream of gas into the ambient atmosphere within the electrostatic field; extruding the fiber-forming liquid into and within the primary stream of gas at a point beyond the point of discharge of the stream of gas and under the influence of the electrostatic field to induce an electrical charge on the extruded liquid, the direction of extrusion being coincident with the direction of the gas flow; attenuating the extruded fiber-forming liquid, breaking the attenuated fiber-forming liquid into discontinuous lengths and at least partially setting the fiber-forming liquid to form discontinuous, electrically charged fibers by maintaining the velocity of the primary stream of gas at the point of discharge at a value greater than the velocity of extrusion of the fiber-forming liquid; and suspending the fibers, completing the setting thereof and depositing the charged fibers in random distribution to form a reticulated, sheet-like, fibrous body by passing the ambient atmosphere upwardly at a velocity greater than the velocity of extrusion of the fiber-forming liquid but lower than the velocity of the primary stream of gas.

13. The method as defined in claim 12 wherein the fiber-forming liquid comprises a solution of a thermoplastic.

14. The method as defined in claim 12 wherein the fiber-forming liquid comprises a solution of an elastomeric material.

15. The method as defined in claim 12 wherein the fibers are deposited on a surface having an electrical charge opposite the electrical charge carried by the fibers.

16. Apparatus for the production of permeable, reticulated, fibrous bodies of fiber-forming organic materials

which comprises a chamber; means including a gas nozzle for passing a stream of gas at a high velocity through the chamber; means including a spraying tube terminating at a point beyond the end of the gas nozzle for extruding a spraying liquid containing a fiber-forming organic material into and within the high velocity stream of gas at a point beyond the end of the gas nozzle thereby attenuating the extruded liquid and breaking the extruded liquid to form discontinuous fibers; means including a source of high potential and an electrode connected electrically to one side of the high potential source and positioned in close proximity to the gas nozzle and the spraying liquid tube for inducing an electrical charge on the extruded fiber-forming liquid and the fibers; and means for collecting the charged fibers.

17. Apparatus for the production of permeable, reticulated fibrous bodies as defined in claim 16 wherein the means for collecting the fibers comprises an electrode connected to the same side of the high potential source.

18. Apparatus for the production of permeable, reticulated, fibrous bodies of fiber-forming organic materials which comprises a chamber; means including a gas nozzle for passing a stream of gas at a high velocity through the chamber; means including a spraying tube terminating at a point beyond the end of the gas nozzle for extruding a spraying liquid containing a fiber-forming organic material into and within the high velocity stream of gas at a point beyond the end of the gas nozzle thereby attenuating the extruded liquid and breaking the extruded

liquid to form discontinuous fibers; means including a source of high potential and two electrodes connected electrically to one side of the high potential source, one of the electrodes being positioned in close proximity to the gas nozzle and the spraying tube for inducing an electrical charge on the extruded fiber-forming liquid and the fibers, and the other of the electrodes being positioned remotely from the gas nozzle and the spraying liquid tube in the path of the stream of gas; and means for collecting the charged fibers.

19. Apparatus for the production of permeable, reticulated, fibrous bodies as defined in claim 18 wherein the first named electrode consists of an open ended cylinder and the second named electrode consists of a porous, conveyor belt.

20. Apparatus for the production of permeable, reticulated, fibrous bodies as defined in claim 18 wherein the first named electrode consists of an open ended cylinder and the means for collecting the charged fibers comprises a porous, collecting surface interposed between the two electrodes.

References Cited in the file of this patent

UNITED STATES PATENTS

55 2,336,745 Manning ----- Dec. 14, 1943

FOREIGN PATENTS

376,598 Germany ----- Dec. 21, 1921

495,737 Belgium ----- Sept. 1, 1950